

Dec. 25, 1928.

1,696,511

H. E. WETHERBEE

METHOD OF TREATING ARTIFICIAL FUELS

Filed Oct. 22, 1925

Fig. 1



Fig. 2



Fig. 3



Fig. 4



Herbert E. Wetherbee

INVENTOR

BY

*H. E. Wetherbee*  
ATTORNEY.

## UNITED STATES PATENT OFFICE.

HERBERT E. WETHERBEE, OF CLEVELAND, OHIO, ASSIGNOR OF ONE-THIRD TO RICHARD F. GRANT AND ONE-THIRD TO HOWARD M. HANNA, BOTH OF CLEVELAND, OHIO.

## METHOD OF TREATING ARTIFICIAL FUELS.

Application filed October 22, 1925. Serial No. 64,125.

My invention relates to improvements in method of treating and forming artificial fuels and to the resultant fuel produced thereby; the object of my invention being 5 to produce a fuel from small sizes of anthracite or bituminous coals, lignite or other carbonaceous material, but preferably from varying small sizes of anthracite, which shall be commercially available for domestic and 10 other use.

Hitherto, difficulty has been experienced in all briquetting processes, with which I am familiar, in getting a suitable binding material in sufficiently intimate contact with the 15 carbonaceous material preparatory to briquetting. This, in many processes, requires a thorough drying of the carbonaceous material, before the binder is applied, in order to remove the water coating adherent to the 20 carbonaceous material and thus enable the binder to make contact therewith. Such drying requires special apparatus and adds materially to the cost of the operation.

It is apparent that a very small amount of 25 suitable binding material, evenly distributed over carbonaceous material and in intimate contact therewith, should suffice to firmly bind the carbonaceous material together upon briquetting. The fault with present processes is that the method or methods used do 30 not evenly distribute the binder over the carbonaceous material, requiring, therefore, an excessive amount of binder in order to cover all the carbonaceous material and therefore 35 unnecessarily increasing the cost.

Accordingly, I have directed my efforts to a method which will, first, bring suitable binding material in intimate contact with carbonaceous material, without drying the 40 carbonaceous material, thereby avoiding the expense of drying the carbonaceous material, and, second, will apply the binding material evenly and uniformly over the carbonaceous material, thereby avoiding the expense 45 of unnecessary binding material.

The spreading action of oil on water is well known. Even oils of great thickness and viscosity will spread almost indefinitely on water. It is also well known that oils even 50 of great thickness and viscosity will, upon agitation with water, break up into exceedingly small particles scattered throughout the water.

I have found that, if carbonaceous material is immersed in water and if oil is put in or on 55 the water and sufficient agitation of the whole is had, the carbonaceous material and the oil will be held in suspension in or on the water and the agitation will enable the particles of carbonaceous material to make frequent and 60 practically continuous contact with the thin films and small particles of oil. Since the carbonaceous material has a greater adhering power for oil than for water, the water adherent to the carbonaceous material will be 65 displaced by an adherent film of oil. Any suitable mixing device or agitator may be used for this purpose. The coating operation progresses rapidly so that a minute film of 70 oil forms over each of the particles of carbonaceous material by almost immediate displacement of the water coating by the oil film, thereby forming a substantially uniform surface oil film on each particle of the carbonaceous material.

Therefore, it is entirely practicable at 75 normal temperatures, to put a thin, substantially uniform surface oil film upon carbonaceous material, even with oils of great thickness and viscosity, by agitation of the carbonaceous material and oil and water as herein described, a result which cannot be obtained by any other process.

I have found that certain oils having the 80 requisite binding qualities may be used as a binder under this method, notably the oxidizing or drying oils, or any oil that will thicken 85 and form a potentially adherent film under atmospheric action alone, or augmented by heat, if desired, in order to hasten the action 90 thereof. A list of such oils includes the various grades of linseed oil, China-wood oil, cottonseed oil, menhaden oil, corn oil, soy bean oil, treated resin oil, asphalt oil or even coal tar products, etc.

I have also found that, in many cases, the binding action of the oil is strengthened and augmented by mixing with or using with the oil other suitable binding material or materials, such as dextrine, resin, etc. In many cases 100 this mixture or use enables me to obtain satisfactory results with the use of less oil than would otherwise be required. This mixture or use of other binding materials with the oil may be accomplished in two ways—

First.—Mixing the other binding material

or materials with the oil before agitating with the carbonaceous material and water as described, in which case the oil film formed on the carbonaceous material carries with it 5 the other binding material or materials.

Second.—Forming first the oil film on the carbonaceous material by agitating the oil with the carbonaceous material and water as described, then draining off the excess water 10 and then treating the oil film on carbonaceous material with a bath containing such other binding material or materials. In this case the other binding material or materials will be taken out of the bath by the adherent action 15 of the oil film for the other binding material or materials and will then be available for briquetting along with the oil film to strengthen and augment the binding power of the oil film.

20 I have also found that many oils, and other liquids not classed as oils, which have the requisite adherent quality to the carbonaceous material but which have little or no binding power, may be used as solvents for binding 25 materials and the resultant solution utilized in the same manner as an oil with binding qualities; for example, asphalt in solvent naphtha, etc.

Any excess water remaining after the adherent film has been formed on the carbonaceous material is then drained off and the product may be introduced immediately to a 30 briquetting machine for producing briquettes of any desired size. These briquettes 35 preferably are subjected to a moderate heating or drying action in order to hasten production and insure oxidation or solidifying of the oil film or binder and the elimination of readily volatile matter therefrom, thereby 40 obtaining satisfactory adhesion of the mass.

While I have above instanced the use of suitable oils and binding material for practicing my invention, I do not wish to be understood as necessarily limiting the same 45 to the drying or semi-drying oils and binding material mentioned, since the same contemplates the use of any oils suitable for this purpose, either alone or in suitable admixture with other oils or binding material or 50 materials, or any suitable fluid binder of negligible miscibility with water or any suitable binder in solution in a fluid of negligible miscibility with water, that will produce a potentially adherent film under the conditions 55 of using the immersed carbonaceous material without artificial drying, and treating the same and briquetting as above described.

I also call attention to the difficulty which has heretofore been experienced in using 60 varying sizes of carbonaceous material, coarser than so-called anthracite culm, for briquetting because proper adhesion of these varying and irregular sizes could not be satisfactorily obtained and such efforts as have 65 been made along these lines resulted in a fuel

that was commercially unsatisfactory, whereas, under my improved process herein described, this difficulty is completely and satisfactorily overcome.

I have shown somewhat diagrammatically 70 in the accompanying drawings one means for practicing the process herein described, wherein:

Figure 1 is an end elevation of a rotatable cylinder or drum. 75

Fig. 2 is a side elevation thereof.

Fig. 3 is a transverse section on line 3—3, Fig. 2, generally indicating the fuel and water levels; and

Fig. 4 is a longitudinal section thereof on 80 line 4—4, Fig. 1.

Throughout the several figures of the drawings I have employed the same character of reference to indicate similar parts.

In the somewhat diagrammatic showing, 85 the rotatable cylinder *c* is mounted on stub-shafts *s*, rotatably supported by the standards *s'* and actuated by the gear *g*. Within the cylinder there are provided a plurality of baffles *b* which are adapted to elevate the fuel particles *f* above the level of the water *w* and its surface coating *a* of agglutinating material, through which the fuel particles are permitted to fall as the cylinder is rotated.

The contents may be supplied by means of the chute *c'* when the hand-hole *h* is rotated to the upper position shown in Fig. 2; this opening thereupon being tightly closed to permit of the agitation of the contents when the cylinder is fully charged. 95

Obviously, upon rotating the cylinder, thorough agitation of the contents is effected, the comminuted material or fuel *f* being carried up by the baffles and dropped through and agitated with the surface coating *a* of 105 agglutinating material for the purpose of enabling the particles of carbonaceous material to make frequent and practically continuous contact with the thin films and small particles of oil distributed on and throughout the water thereby, and effecting an even distribution of the agglutinating material throughout the mass of the finely sub-divided fuel *f*.

It will be understood, of course, that the proportions in the drawing, and particularly, the stratum *a* of agglutinating material, are merely illustrative, and do not represent operating conditions, relative quantities or 115 volumes, and sizes of parts.

As a formula exemplifying the practice of my improved process, I may state that with a given quantity of the finer breaker products of anthracite, comprising roughly a major imbedding content of culm and twenty per cent (20%) each of No. 1, 2 and 3 buckwheat, for example, I combine from approximately one half of one per cent to approximately two and one half per cent, by weight, according to the binding characteristics of the 120 125 130

binding material used, by treatment as herein described, and thereby produce a briquette of satisfactory strength and burning qualities at a comparatively low cost.

5 It is my understanding that the oxidized or solidified oil binders will burn approximately the same as the adherent carbonaceous particles. In consequence, briquettes can be produced in accordance with my invention which are equally satisfactory for purposes of transportation and combustion, which is not the case where some classes of binders are used.

10 My instant process has the obvious advantages and economies of—

First.—Elimination of drying of the carbonaceous material;

Second.—Even and continuous distribution of the binding material on the carbonaceous material in intimate contact therewith, thereby requiring the use of a minimum amount of binding material and saving the expense of additional and unnecessary binder required under other methods and processes;

25 Third.—Making it commercially practicable to use varying sizes of carbonaceous material.

Accordingly, the briquettes produced in accordance with my instant improvement are 30 low in cost while satisfying every commercial requirement.

Having now described the preferred procedure for practicing my instant invention, I claim as new and desire to secure by Letters Patent, together with such modifications as to procedure, proportions and ingredients used, as may be supplied by one ordinarily skilled in the art, the following:

1. In a method for treating comminuted 40 materials preliminary to briquetting the same, the step of subjecting the particles thereof while in moistened condition to the action of a moisture displacing filming oil binder, substantially as set forth.

45 2. The method of producing artificial fuel which consists in immersing sub-divided carbonaceous material in water, adding thereto a binding material productive of a potentially adherent film upon the particles of said carbonaceous material, agitating the same under the conditions herein described, draining off the excess water, and subjecting portions of the mass to pressure for inducing adhesion thereof, substantially as set forth.

55 3. The herein described method of treating particles of carbonaceous material to insure adhesion thereof, which consists in immersing the same in water in or on which has been placed a sufficient amount of binding material that will produce a potentially adherent film on said carbonaceous material, agitating the same under the conditions herein described, draining off the excess water and subjecting bodies of the mass to pressure

65 to induce adhesion thereof, substantially as set forth.

4. The herein described method of treating particles of carbonaceous materials to insure adhesion thereof, which consists in immersing the same in water, in or on which has been placed a sufficient amount of agglutinating oil to produce a potentially adherent film on the carbonaceous material, agitating the same under the conditions herein described, draining off the excess water and 70 subjecting bodies of the mass to pressure to induce adhesion thereof, substantially as set forth.

75 5. The herein described method of treating comminuted fuels, which consists in immersing the fuel particles in water, spreading upon the surface of the water a thin stratum of agglutinating material having negligible miscibility, causing the fuel particles to pass through said stratum to effect 80 filming thereof, draining off the excess water, and subjecting small masses of the fuel particles to pressure sufficient to insure their adhesion, substantially as set forth.

85 6. The herein described method of treating fuels, which consist in spreading upon the surface of a body of water, a small quantity of filming agglutinating material, having negligible miscibility, passing through the stratum of said material a quantity of 90 carbonaceous material in finely divided and moistened condition, whereby the moisture is displaced by a film of said agglutinating material, draining off the excess water and briquetting the carbonaceous material, substantially as set forth.

95 7. The herein described method of applying an agglutinating oxidizable oil to sub-divided fuel particles, which consists in spreading an oxidizable or potentially solidifying oil of negligible miscibility upon the surface of a body of water, passing the fuel particles through the thin stratum of oil while in moistened condition to insure the 100 filming action of the oil, draining off the excess water, briquetting the fuel particles and oxidizing or solidifying the oil to obtain the coalescence of the fuel particles, substantially as set forth.

105 8. The herein described method of treating fuels, which consists in immersing the sub-divided fuel in a fluid medium, adding to said fluid medium a small quantity of filming agglutinating oxidizable oil, agitating the sub-divided fuel into contact with said agglutinating material whereby a film is formed 110 upon the particles thereof, draining off the water of immersion, and subjecting small masses of the treated sub-divided fuel to pressure, substantially as set forth.

120 125 9. The herein described method for coalescing irregular small sizes of anthracite and the like, which consists in treating a mass

thereof in moistened condition with a suitable filming oxidizable oil binder to displace the water, and thereafter effecting the drying or solidifying of said oil to insure its adherent 5 action, substantially as set forth.

10. The herein described artificial fuel, comprising sub-divided carbonaceous material and a binder less than two (2%) per cent of the total weight thereof.

10 11. A briquette, comprising a body of comminuted material and a binder therefor less than two (2%) per cent of the total weight of said material filming the particles thereof.

15 12. The herein described artificial fuel, comprising sub-divided carbonaceous material and a binder not in excess of one (1%) percent of the total weight of the product.

13. The herein described artificial fuel, 20 comprising varying small sizes of anthracite or the like coalesced by a binder not in excess of one and one-half (1½%) percent of a filmed agglutinant, by weight.

14. The herein described artificial fuel, comprising a coalesced mass of carbonaceous material and its filmed agglutinant; the latter approximating one (1%) percent of the total weight.

15. The herein described artificial fuel comprising coalesced carbonaceous material 30 with a binder consisting primarily of less than two (2%) per cent of a filming agglutinating oil.

16. The herein described artificial fuel comprising coalesced carbonaceous material 35 with a binder consisting exclusively of a filming agglutinating oil less than two (2%) per cent of the total weight thereof.

17. The herein described artificial fuel comprising varying small sizes of coal products coalesced exclusively by a filming oil binder approximating one (1%) per cent of the total weight.

In testimony whereof I do now affix my signature.

HERBERT E. WETHERBEE.